

# UNITED STATES PATENT OFFICE.

HENRY K. SANDELL, OF CHICAGO, ILLINOIS, ASSIGNOR TO HERBERT S. MILLS, OF CHICAGO, ILLINOIS.

## WHITE METAL ALLOY

1,248,925.

Specification of Letters Patent. Patented Dec. 4, 1917.

No Drawing.

Application filed June 18, 1917. Serial No. 175,371.

To all whom it may concern:  
Be it known that I, HENRY K. SANDELL, a citizen of the United States, residing at Chicago, in the county of Cook and State of Illinois, have invented a new and useful improvement in White Metal Alloys, of which the following is a specification.

My invention relates to certain improvements in white metal alloys and will be fully understood from the following specification.

For the preparation of my new alloy the following procedure is adopted:

10 parts by weight of bismuth together with 10 parts by weight of tin is melted in any suitable apparatus, preferably in a crucible which may be covered to exclude the atmosphere, the molten mass is permitted to cool very slowly until it reaches a temperature just above its setting temperature. At the moment before solidification or setting begins there is added 10% of mercury, under which conditions the mercury may be caused to dissolve itself in the mixture.

25 This primary alloy is then permitted to set.

20 parts by weight of zinc are now melted in a suitable crucible as, for example, the covered crucible above referred to, and the zinc is permitted to cool to a point just above its solidification temperature. The primary alloy of bismuth, tin and mercury is now added to the zinc and this mixture is permitted to set. The secondary alloy is now complete.

35 The third step of the process consists in

melting in the covered crucible 50 parts by weight of copper, the temperature of the molten copper is slowly reduced and just before solidification begins, the secondary alloy prepared as above is added to the 40 copper.

My alloy of mercury, bismuth, tin, zinc and copper is now complete and may be cast and otherwise fabricated as desired.

My improved alloy is a white metal which 45 takes a brilliant polish and holds it on exposure to the atmosphere. Its melting point is slightly below that of copper, its tensile strength is relatively low and it is relatively brittle, giving a fracture similar to that of 50 glass.

What I claim is:

1. An alloy comprising 10 parts by weight of mercury, 10 parts by weight of bismuth, 10 parts by weight of tin, 20 parts by weight 55 of zinc, and 50 parts by weight of copper.

2. The method of preparing the above-described alloy which comprises forming the primary alloy of bismuth and tin, adding to such primary alloy while the same is 60 at a temperature not substantially exceeding its melting point the required amount of mercury, adding the said primary alloy to the molten zinc at a temperature not exceeding its melting point, thus forming a 65 secondary alloy, and adding such secondary alloy to molten copper at a temperature not substantially exceeding its melting point to produce the final alloy.

HENRY K. SANDELL.